

Oct. 22, 1946.

W. H. McDOWELL

2,409,984

METHOD OF TREATING WATER RESISTANT PAPER

Filed May 15, 1945



WENDELL H. McDOWELL

INVENTOR

BY *W. M. Perrins*  
*Daniel J. Mayne*  
ATTORNEYS

## UNITED STATES PATENT OFFICE

2,409,984

METHOD OF TREATING WATER  
RESISTANT PAPERWendell H. McDowell, Rochester, N. Y., assignor  
to Eastman Kodak Company, Rochester, N. Y.,  
a corporation of New Jersey

Application May 15, 1945, Serial No. 593,829

6 Claims. (Cl. 117—62)

1

This invention relates to a method of treating melt coated, water resistant paper in which the melt coating of the paper is treated with only enough of a lower monohydroxy alcohol to wet the surface of the coating and is then evaporated therefrom.

Recently the coating of paper with hot fluid melts consisting of a cellulose ester and a plasticizer has become of interest, particularly for the preparation of water resistant paper suitable for photographic purposes. This melt coated paper is described in U. S. application, Serial No. 553,804, of Hollis T. Galley, filed September 12, 1944, and in U. S. applications, Serial Nos. 512,051 and 512,052 of Salo and Vivian, filed November 27, 1943 which have matured into Patents Nos. 2,387,773 and 2,387,774. In the use of photographic paper for picture making it is often desirable after a photographic print has been developed, fixed, and washed to pass it over hot metal drying surfaces such as heated to a temperature of 200-260° F. whereby the photographic paper is quickly dried, thus saving time and contributing to the quality of the product obtained. As long as the hot surfaces are maintained below the melting temperature of the coating, drying of the ordinary-type photographic paper by this means is very satisfactory.

In those cases, however, where melt coated paper has been employed as the support for a photographic emulsion, it has been found that sticking of the paper to the hot metal surface may occur in the drying operation. The melt-coated water resistant paper ordinarily contains a coating of cellulose acetate butyrate plasticized with a stable, high-boiling material, such, for instance, as a mixture of dibutyl sebacate and butyl stearate or of di-2-ethyl hexyl-phthalate and butyl stearate. Because of the nature of this coated material, methods of drying the photographic paper less convenient than the use of hot surfaces have been necessary.

Heretofore where thermoplastic sheeting has exhibited sticking properties, such as upon binding that material together for shipping or storage, it has been suggested that if the surface of the sheeting was roughened or microscopically pitted, sticking would not occur. Although methods of this nature might be useful for some types of thermoplastic sheeting, the presence of a roughened surface on photographic paper is not particularly desirable. Other methods such as heating the paper in a hot chamber and then cooling, prior to packing have been considered. However, in practice, difficulties are met with

2

which decrease the advantages in the use of such a procedure. In other cases where thermoplastic sheeting has exhibited sticking, thin layers of cellulose esters from solution of the esters in volatile solvents have been applied thereto. In the present situation this merely adds to the weight of the photographic paper and also presents other difficulties, such as the effect of the volatile solvents on the melt coating which has already been applied. Therefore, none of the methods which has previously been considered for cellulose ester sheeting have been regarded with too much favor for inhibiting the adhesive-ness of melt coatings.

15 One object of my invention is to provide a method of treating melt coated paper so as to prevent sticking of that paper to hot metal drying surfaces. Another object of my invention is to provide a method of treating melt coated paper 20 to inhibit sticking of that material to hot surfaces, which method does not increase the weight or alter the surface characteristics of the melt coating. A further object of my invention is to provide a simple, easily operated method of treating 25 melt coated paper to decrease its sticking properties.

I have found that melt coated paper which is 30 dampened or slightly wetted with a lower aliphatic alcohol, which alcohol is then evaporated therefrom provides a surface which will not stick to hot metal drying surfaces such as are ordinarily employed in drying photographic prints or in ferrotyping operations. In its broadest aspects my invention comprises the treatment of paper 35 which has been melt coated on at least one surface with a small amount of alcohol, on that surface, which is preferably applied only in an amount insufficient to run off the same. The melt coated paper the surface of the melt coating of which 40 is thus dampened with the alcohol is preferably almost immediately treated to drive off the alcohol such as by passage of the so-dampened paper through a heated chamber. The surface so treated will not become tacky upon contacting 45 with a hot metal drying surface such as having a temperature of 200-260° F. and no adhesion to the metal takes place. In the process in accordance with my invention only enough alcohol is employed to wet the surface and, therefore, there 50 is no substantial washing out of any of the materials which are present such as would occur by an immersion operation.

One procedure which might suggest itself as being remedial of the sticking characteristics of 55 melt coated paper would be to employ a melt coat-

ing composition in which the amount of plasticizer employed is reduced to the barest minimum. This, however, introduces difficulties into the melt coating operation, as the presence of sufficient plasticizer to insure a good melt is necessary for the efficient and speedy coating of paper. With the use of restricted amounts of plasticizer the speed of the coating operation is restricted in that drying lines appear on paper at certain speeds, if the melt is not of the most desirable type. My process as adaptable to preventing the sticking of melt coated papers even though the amount of plasticizer employed in the melt coating operation has been as much as 50% based upon the cellulose ester which is employed in the melt composition.

Ordinarily paper is melt coated with a composition consisting of cellulose acetate butyrate having a high butyryl content, such as a butyryl content of 50% and a substantial proportion of a plasticizer which is sufficiently solvent of the cellulose ester to form a good melt but which will not give tackiness after the melt coating has cooled. A good example of a composition useful for melt coating is a mixture of a cellulose acetate butyrate having a butyryl content of approximately 47%, and 33½%, based on the weight of the cellulose ester, of a plasticizer consisting of three parts of dibutyl sebacate and two parts of butyl stearate. This composition is heated to a temperature of 160-170° C. and may be applied to paper in any desired manner giving a good coating thereon. For instance, the melt coating may be applied by a bead application in which the paper after coating is run over a blade for smoothing purposes while still in a plastic condition. The paper which is thus coated may either have been first baryta coated or the melt coating may have been applied first, followed by the application of a baryta coating thereto.

The alcohol treatment may be imparted to the melt coated, water resistant paper either before, during, or after the application of a photosensitive emulsion thereto. For instance, after a paper has been melt coated the paper may be passed through a heated chamber, such as heated to 190° F., in which chamber the alcohol is flowed out onto the paper and almost immediately evaporated therefrom. In order to increase the speed of removal of the alcohol from the paper thus coated, both the coating operation and the evaporating operation may take place within the heated chamber for the sake of convenience.

After the paper has been treated with alcohol in accordance with my process photographic emulsion may be applied thereto, preferably on the side of the paper to which the alcohol has not been applied (providing only one side of the paper was treated). If the photographic emulsion had first been applied to the paper before, or simultaneously with the alcohol treatment, it is ready after evaporation of the alcohol therefrom for use for photographic purposes. After the paper has been exposed, it may then be developed, fixed, and washed in the conventional manner whereupon it may be passed over a hot metal surface such as a metal drum having a temperature of 200-260° F., the side of the paper which had been treated with the alcohol being contacted with the hot metal. The paper which had been treated in accordance with my invention readily dries and falls away from the hot metal surface with which it contacts.

Although the invention has been described using ethyl alcohol as the wetting liquid, it is to be

understood that other lower aliphatic alcohols may be employed for this purpose, the lower monohydroxy aliphatic alcohols of 1-4 carbon atoms being especially useful as ease and speed of removal of the alcohol is a consideration. It is ordinarily desirable to employ methyl or ethyl alcohol for this treatment.

The following example illustrates my invention:

Paper which had been baryta coated and then coated on both sides with a hot melt-coating of cellulose acetate butyrate, dibutyl sebacate, and butyl stearate as described in Salo and Vivian Patent No. 2,387,773, was passed into an enclosed chamber and through a bead type hopper applicator therein, this type applicator being illustrated by the drawing of this application. The paper 1 is passed between press roll 2 and applicator roll 3, the side of the paper contacting the applicator roll being that which is not baryta coated. The applicator roll dips into a body of commercial ethyl alcohol 5, contained in the vessel or hopper 4 and in turn moistens the surface of the melt coating which it contacts.

The enclosed chamber in which the applicator is found and through which the paper was passed was maintained at a temperature of 160-180° F. by the passage of a current of warm, dry air therethrough. The hopper containing the alcohol was jacketed and cool water was passed through the jacket to minimize evaporation of alcohol from the hopper.

Forty-two thousand feet of paper 3½ feet wide were put through the applicator which took approximately 400 pounds of alcohol to moisten the melt-coated surface. After moistening in the applicator the paper was almost immediately freed of alcohol due to the warm air circulating in the chamber within which the treatment took place.

The paper was then coated on the baryta coated side under darkened conditions with a gelatino-silver halide emulsion, preferably after first subbing the paper. After exposing the paper it was processed by developing, fixing and washing and was dried by running over a hot metal ferrotyping roll, the alcohol-treated side of the paper contacting the roll. The paper dried readily without sticking to the metal surface.

Instead of applying the alcohol by the bead method, it may be applied by any method by which the surface of the melt coating is moistened with the alcohol, such as by flowing or spraying the alcohol on to a rapidly moving paper sheet which has been melt coated. The application of alcohol may be separated from the drying or evaporating means, the paper in this case after the application of the alcohol, being led into evaporating conditions.

The alcohols preferred for use are those of fairly high concentration such as 93-100% alcohol. However, more dilute alcohol may be employed within the scope of our invention. The water, however, dilutes the alcohol and thus necessitates the handling and the evaporation of a larger quantity of liquid than in those cases where a more concentrated alcohol is used. As a general rule the alcohol employed should be of at least 80% concentration.

The amount of alcohol which is applied to the surface of the melt-coating need only be sufficient to dampen or moisten that surface. Greater quantities will tend to run off of the paper and would be uneconomical in the excessive use of alcohol. I have found that the application of 2-4 pounds of alcohol per 1000 square feet of

paper is the best range for operation although the treatment of the surface with alcohol and evaporation thereafter is within the purview of my invention.

My invention includes not only the treatment of the melt-coated surface of paper with alcohol but also the evaporation of the alcohol therefrom. In practical operation it is desirable to subject the paper to an elevated temperature, such as by means of a current of warm air to accomplish the removal of the alcohol fairly rapidly. Where time is not of importance the drying or removal of the alcohol may be accomplished as desired, such as by exposing the treated paper to the air for the desired time. Any drying operation compatible with the conditions here may be employed for the evaporation of the alcohol from the surface moistened therewith.

I claim:

1. A method of treating the surface of paper containing a melt coating of a cellulose ester and a plasticizer to inhibit tackiness when contacted with a hot surface which comprises contacting at least one surface of paper melt coated with a mixture of a cellulose ester and a plasticizer with only sufficient alcohol of 1-4 carbon atoms to wet the same, and evaporating the alcohol from that surface.

2. A method of treating at least one surface of paper containing a melt coating of a cellulose ester and a plasticizer which comprises contacting at least one surface of paper melt-coated with a mixture of a cellulose ester and a plasticizer with only sufficient ethyl alcohol to wet

the same, and evaporating the alcohol from that surface.

3. A method of preventing melt coated paper from sticking to hot drying surfaces which comprises treating the surface of the paper containing a melt coating of cellulose acetate butyrate and a plasticizer thereon with only sufficient lower monohydroxy aliphatic alcohol of 1-4 carbon atoms to wet the same and evaporating the alcohol from the surface of the coating.

4. A method of preventing melt coated paper from sticking to hot drying surfaces which comprises treating the surface of the paper containing a melt coating of cellulose acetate butyrate and a plasticizer thereon with only sufficient ethyl alcohol to wet the same and evaporating the alcohol from that surface.

5. A method of treating melt-coated paper, which has been baryta coated and then melt-coated with a mixture of cellulose butyrate and a plasticizer which comprises treating the surface which has not been baryta coated with only sufficient ethyl alcohol to wet the same and evaporating the alcohol from that surface.

6. A method of treating the surface of paper containing a melt coating of a cellulose ester and a plasticizer to inhibit tackiness when contacted with a hot surface, which comprises contacting at least one surface of paper melt coated with a mixture of a cellulose ester and a plasticizer with only sufficient methyl alcohol to wet the same and then evaporating the alcohol from that surface.

WENDELL H. McDOWELL.